

3,681,261

**RESISTORS, COMPOSITIONS, PASTES, AND  
METHOD OF MAKING AND USING SAME**

Daniel W. Mason, West Peabody, Mass., and Bernard Greenstein and John M. Woulbroun, Toledo, Ohio, assignors to Owens-Illinois, Inc.

No Drawing. Filed July 27, 1970, Ser. No. 58,740  
Int. Cl. B44d 1/02; H01b 1/06

U.S. Cl. 252—514

7 Claims

**ABSTRACT OF THE DISCLOSURE**

Palladium oxide or other metal oxide resistors for microelectronic circuitry are provided with a high degree of reproducibility and stability by first concentrating to powder form a liquid mixture of a resistor metal-organo metallic compound, at least one other stabilizer metal in organometallic form, and an anti-agglomerating agent which will not burn off during processing to final resistor form. The powder is then alloyed and the resistor metal oxidized. The resulting alloy is then formed into a resistor paste by admixing it with a glass binder (either before or after oxidation) and a liquid carrier vehicle. The paste is printed in the desired pattern, dried and fired to produce the resistor in final form.

This invention relates to electronic resistors. More particularly, this invention relates to electronic resistors, compositions, pastes, and methods of making and using same particularly within the environment of microelectronic circuitry.

The art has long known of the value of palladium oxide (PdO) for use as a resistor material, particularly in microelectronic circuitry. Generally speaking, palladium oxide is formed into a resistor by admixing palladium with a glass binder and organic vehicle to form a printing paste. In the case of microelectronic circuitry, the paste is then printed onto a dielectric substrate such as aluminum oxide or the like by the use of a screen or mask of the desired mesh and formed to provide the desired pattern. The patterned design is then fired in air to oxidize the Pd to PdO and form the ultimate resistor lamina.

In order to increase the negative temperature coefficient of resistivity (hereinafter referred to as TCR), to regulate ultimate resistivity, and to render the stability of the PdO system acceptable, certain metals are employed in admixture with the palladium in the paste. Such metals, which are referred to hereinafter as stabilizers, are those which do not oxidize at the temperatures used to fire the printed paste.

Many problems attend these prior art PdO resistor systems. One major problem is the great sensitivity of these systems to the firing process as a whole. Slight fluctuations or variations in the firing temperature, for example, greatly changed the resistivity of the resulting product. Air flow and firing times are further variables to which the ultimate characteristics of the final product are extremely sensitive. Such sensitivity, of course, renders these PdO systems extremely difficult to reproduce. Not only is reproducibility low, but for some reason, not entirely understood, stability is also very low.

The term "stability" is well understood in the art and is used herein in accordance with this well known meaning. That is to say, stability defines that characteristic of a resistor which enables it to maintain its resistivity within tolerable limits over extended periods of time and use.

While the stabilizer metals used in admixture with the palladium oxide generally provide commercially tolerable stability to the system, they are generally found to detri-

mentally increase the TCR of the systems, usually far above the  $\pm 0$  p.p.m./° C. level ideally desired. In some instances, especially when Ag is used, stability must be sacrificed for acceptable TCR while, on the other hand, 5 TCR must be sacrificed for acceptable stability. In almost all instances, reproducibility, regardless of the metal stabilizers used, is detrimentally low.

In order to overcome these problems, the art has sought out many solutions. Some have sought to use various additional additives to improve the system. Others have sought to alter the starting materials employed such as by employing finely divided palladium oxide in the paste or initially employing crystalline palladium or its oxide within critical particle sizes and surface areas. Others used 10 combinations of the above solutions or turned completely from the PdO system to seek other resistive metal oxide systems which might have higher stability and/or reproducibility. In many instances, only a modicum of success was actually achieved. In many other instances, the manufacturer was rendered so expensive as to make it economically undesirable.

It, therefore, is apparent from the above that there exists a definite need in the art for a PdO or other resistive metal oxide system which is highly reproducible, 15 has high stability, exhibits excellent TCR's, produces high quality resistors, and is economical to manufacture.

It is a purpose of this invention to fulfill this need in the art. Generally speaking, this invention fulfills this need by providing a resistor composition and/or paste which is uniquely formed in a manner which insures optimum alloying of the metals and controlled homogeneous oxidation of the Pd or other resistive metal prior to firing, to the extent that the resistivity characteristics are not detrimentally sensitive to air flow, time, and temperature variations during firing; thus to provide a highly stable, reproducible resistor for good quality. In addition, because of the optimum alloying and other factors, low TCR's are obtainable.

Basically, the resistor compositions are formulated in accordance with this invention by:

(a) Forming an admixture of a resistive metal-organo metallic compound, at least one metal stabilizer in organometallic form and an anti-agglomerating agent which will remain in the system throughout processing;

(b) Heating the admixture at a sufficient temperature and for a sufficient period of time to drive off the organo-constituents and concentrate the admixture to a powder; and

(c) Heating the powder at a sufficient temperature and for a sufficient period of time to alloy said metals and in some instances to oxidize the resistive metal.

The above-described resistor compositions may be employed in a wide variety of ways and environments for their resistive properties. Any of these ways and environments, conventional in the art, are contemplated by this invention. As alluded to hereinabove, a preferred way in which these resistor compositions may be used is to formulate them into printing pastes and print them on appropriate substrates for use in microelectronic circuitry.

Such pastes are formed in accordance with this invention by admixing the resistor composition in powder form with a conventional glass binder and in some instances oxidizing the resistive metals at this point. Thereafter the 55 oxidized mixture is added to a liquid organic vehicle. The resulting paste may then be screen printed in accordance with conventional techniques in a desired pattern, dried and fired to produce the final resistor lamina. The resistors so formed generally exhibit a stability factor of less than 60 about  $\pm 1\%$  drift during normal load life (e.g., 1000–10,000 hours) and a reproducibility usually on the order of about  $\pm 20\%$  of the specified resistivity.

Generally speaking any one or a combination of the conventional resistive metals may be used in the practice of this invention. Examples of such metals include palladium, rhodium, iridium, ruthenium, indium, and mixtures thereof. Because of the economic advantages, ease of processing, good stability, and good reproducibility, the palladium oxide system, and thus palladium, is preferred for the purposes of this invention.

Any of the well known stabilizing metals may be used in the practice of this invention. Generally, these metals are chosen for their inertness to oxygen at the operating conditions of this invention. Although only one of these metals may be employed, it is preferred to use at least two metals together in amounts which have been found to synergistically minimize their effect upon TCR. Examples of these stabilizing metals include silver, gold, and platinum. Examples of preferred admixtures in parts-by-weight ratio for minimization of effect on TCR include Ag:Au, about 4:1-1:4; Pt:Ag, about 8:1-1:8; and Pt:Au, about 8:1-1:8. Particularly preferred for the purposes of this invention is the Ag:Au admixture since it is found that this admixture when alloyed with Pd will form a single phase alloy, thus further minimizing the effect of firing on the system.

Any of the well known organo-metallic compounds of the above metals may be used, provided that they are capable of being concentrated from admixture to a powder form. Such, of course, generally assumes that the organo-metallic compounds are liquids or are solids dispersed or dissolved in conventional liquid media. In addition, the organo-metallic compounds contemplated are those from which the organic constituents are capable of being driven off during concentration and/or to a lesser extent, during firing.

Preferred organo-metallics for the purposes of this invention are the well known metal resinate. Particularly preferred among the metal resinate are the conventional metal mercaptans because of the ease by which they may be concentrated to a substantially homogeneous powder, their availability and the like. Such mercaptans are well known and may be obtained, for example, from Englehard Industries, under such trade designations as Gold #8300, a mercaptan having 28.0% by weight Au; Rhodium #8826, a mercaptan having 10.0% by weight Rh; Platinum #9450, a mercaptan having 26.0% by weight Pt; Palladium #7611, a mercaptan having 20.0% by weight Pd; Iridium 8057, a mercaptan having 24.0% by weight Ir; and Silver 9144, a mercaptan having 30.0% by weight Ag.

Other resinate useful include the balsam based resinate examples of which, obtainable from the indicated company, include Gold A-1118 and A-1119, a balsam having 24% by weight Au and 12.0% by weight Au, respectively; Rhodium A-1120, a balsam having 5% by weight Rh; Platinum A-1121, a balsam having 12.0% by weight Pt; Palladium A-1122, a balsam having 9.0% by weight Pd; Iridium A-1123, a balsam having 6.0% by weight Ir; and Ruthenium A-1124, a balsam having 4.0% by weight Ru.

Specific examples of the mercaptides of the above resistive and stabilizer metals include metallic ethyl mercaptide, n-octyl mercaptide, benzyl mercaptide, tertiary amyl mercaptide, tertiary hexadecyl mercaptide and the like. Other examples include the chlorometallic mercaptide such as chlorometallic tertiary hexylmercaptide-methyl sulfide, chloro-metallic (e.g. Pt) methyl mercaptide-propyl sulfide, chloro-metallic isoamylmercaptide methyl sulfide and the like.

The anti-agglomerating agents useful for the purposes of this invention are those conventional materials which are inert to the system and which will not burn out at alloying and/or firing temperatures. Such anti-agglomerating agents are usually of a fine particle size, e.g., less than about 5 microns. Examples of these agents include: ultrafine alumina, ultrafine  $TiO_2$ , and other ultrafine refrac-

tories. Preferred for the purposes of this invention is ultrafine silica which is purchasable under the trademark Cab-O-Sil L-5.

This invention also envisions the use of other additives, known in the art, to the above ingredients in order to enhance, in a known fashion, one or more of the desired characteristics of the system.

As stated, the above resistor compositions of this invention are formed by first admixing the requisite amounts of resinate together in liquid form. Homogeneity is desired and thus thorough mixing of the resinate should be effected. For the preferred palladium systems contemplated, the resinate are admixed in proportions so as to present about 5-95% by weight of the metal content as palladium. Preferably, the Pd content is 15-75% of the total metal content and more preferably from 20-65%. The remainder of the metal content usually consists of one or more stabilizer metals.

To this homogeneous admixture of resinate there is added, with continuous stirring, an anti-agglomerating agent. Generally speaking this agent is added in an amount sufficient to prevent any substantial amount of agglomeration from taking place during the later alloying step. Although not limited to any particular theory, it is felt that the use of this agent greatly aids in improving the stability and reproducibility of the system.

The exact amount of anti-agglomerating agent used will, of course, vary, depending upon the system used and the type of agent employed. Generally speaking, however, the agent is used in an amount of about 0.5 to about 15% by weight of the metal powder formed upon concentration. When a PdO system is employed and the agent is finely divided silica, about 5% agent by weight of the metal powder is preferred.

After addition of the anti-agglomerating agent, the mixture is heated with stirring for a sufficient period of time and temperature to concentrate the mixture to a powdery solid. Generally speaking, and when the resinate are mercaptide based, heating to powder is conducted at about 100-200° C., preferably at about 125° C., for about 3-4 hours. The resulting powder is an extremely homogeneous mixture of the metals having the anti-agglomerating agent dispersed therein and from which substantially all of the organic constituents have been removed.

The powder so formed is heated at a temperature and for a period of time sufficient to alloy the metal. Because of the homogeneity and non-agglomerated nature of the starting powder, alloying is homogeneous and thus optimized. The resulting powdered alloy is, therefore, an anti-agglomerated homogeneous powder ready for further processing.

The temperature at which alloying is effected will depend upon whether or not oxidation of the resistive metal is desired at this point. In those instances where the resistive metal is to be oxidized, the process will take place in air and the temperature of alloying will be sufficiently high to permit the oxide to form but not so high as to prevent oxidation from taking place. In a palladium system, such a temperature is about 650-750° C. Of course, alloying time will be extended to insure the requisite amount of oxidation. In those instances where oxidation is not to be effected at this point, but rather effected in a separate step, alloying is accomplished either in an inert atmosphere and/or at temperatures at which oxidation of the resistive metal will not occur.

In preferred embodiments of this invention, the oxidation is effected in a separate step. Preferably, the second oxidation step is effected either immediately following the alloying step, or after the addition to the alloy of the glass binder when a paste is to be formed.

In those instances where oxidation is effected immediately after alloying, alloying is preferably carried out at a temperature higher than that at which any substantial amount of oxidation of the resistive metal will occur. For the preferred Pd system such a temperature is usually

above about 725° C. and usually from 800–900° C. Since alloying is time-temperature dependent, sufficient time should be allotted to allow for complete alloying. About 1–48 hours, depending upon the size of the batched powder, is usually sufficient for this purpose. After alloying is effected, the temperature is then lowered to a convenient oxidizing temperature, and if an inert atmosphere was employed, air is pumped into the environment to effect the oxidation step. Oxidation is also time-temperature dependent and thus sufficient time is allotted preferably for as complete oxidation of the resistive metal as possible. Generally speaking, the preferred range of oxidation temperatures for the PdO system is from about 300° C.–725° C., and more preferably, about 650–725° C. Times will vary but generally speaking, times of about 1–48 hours are found to be sufficient.

In those instances, as stated above, where the alloys are to be made into pastes, oxidation may be effected after the alloyed powder is admixed with the glass binder of the paste composition. Generally speaking, this is accomplished by ball-milling a particulate glass binder having an average particle size less than about 5 microns with the powdered, anti-agglomerated alloy. After these ingredients are thoroughly ball-milled and thus admixed, the mixture is subjected to oxidizing conditions (i.e., the oxidation times and temperatures set forth hereinabove) to effect oxidation of the resistive metal in the alloy. Although not limited to any particular theory, it is believed that oxidation at this point preferably to as complete an extent as is possible, optimizes reproducibility and stability and minimizes TCR's since the substance oxidized will be that presented to the firing step without any further physical comminution or the like. Where complete oxidation is effected, reproducibility is optimized since substantially no oxidation can occur during firing. In this respect the term "complete oxidation" is being used to define that point at which substantially all of the resistive metal presented for oxidation is oxidized. Thus this term is being used to define that degree of oxidation at which substantially no further oxidation will take place during firing. This is not to say that all of the resistive metal in the system is oxidized, since in many instances, alloying masks some of the alloy from oxidation.

In a preferred embodiment wherein the Pd system is employed, oxidation after glass binder addition is conducted between about 300 to 450° C. for a period of about 8 to 48 hours. Using such conditions, oxidation is found to be substantially complete.

With respect to the degree of oxidation effected, resistivity can be controlled by the amount of oxidation, and thus it is contemplated that oxidation, regardless of how it is effected, does not necessarily have to be complete, but rather only to a degree sufficient to afford the desired resistivity. This invention, however, contemplates in its preferred form and regardless of how oxidation is accomplished, the use of oxidizing conditions such that as complete oxidation (as defined above) as possible is obtained. This insures maximum reproducibility while ultimate resistivity is controlled by the amount of resistive metal initially employed and/or the alloying cycle chosen.

As stated hereinabove and regardless of which oxidation procedure is employed, the resistor compositions of this invention may be formulated into printing pastes, especially for use in microelectronic circuitry printing. Such printing pastes may be formed by any conventional technique. Generally speaking a preferred technique is to admix the alloyed powder with a glass binder (before or after oxidation as described) and a suitable volatile organic liquid binder.

Glass binders for use in the pastes of this invention are conventional and generally speaking, any of these conventional binders may be employed. Examples of such binders include the boro-silicates and particularly the lead-alumina-borosilicates. A particularly preferred glass binder, in particulate form, having an average particle size

of less than about 5 microns, is represented by (in weight percent):

|                                      | Percent        |
|--------------------------------------|----------------|
| SiO <sub>2</sub> -----               | About 8 to 12  |
| B <sub>2</sub> O <sub>3</sub> -----  | About 20 to 30 |
| Al <sub>2</sub> O <sub>3</sub> ----- | About 2 to 7   |
| ZnO -----                            | About 20 to 30 |
| PbO -----                            | About 30 to 40 |

10 The organic liquids used are conventional and generally speaking, any one of these well-known liquids may be employed. Examples of these liquids include butyl Carbital acetate (diethylene glycol monobutyl ether acetate), iso-amyl salicylate and mixtures thereof. A particularly preferred liquid vehicle is a mixture of 2 parts by weight butyl Carbital acetate to 1 part by weight iso-amyl salicylate.

15 In a preferred manner of formulating the pastes contemplated by this invention, the alloy and glass binder are first thoroughly admixed as by ball-milling and thereafter the resulting admixture is stirred and roller milled into the requisite amount of liquid vehicle to provide a printing paste of the desired consistency. The paste so formed may then be printed in a desired pattern using a conventional screen or mask. Thereafter, the printed design is dried and fired to produce the final resistor, usually upon a dielectric substrate. Drying after printing may be effected by either air drying and/or oven drying, usually at a temperature of about 100–125° C. for about 5–10 minutes. Firing is usually accomplished thereafter at a temperature of about 700° C. ±50° C. (for the PdO system) using a heat-up peak and cool-down cycle of about 20–60 minutes with firing at peak temperatures for about 2–15 minutes.

20 25 30 35 40 As stated hereinabove, the resulting printed resistors of this invention are found to be highly reproducible, have excellent stability, and generally have TCR's less than ±500 p.p.m./° C., usually less than ±200 p.p.m./° C., and in some instances, substantially close to 0 p.p.m./° C.

The following examples are presented as illustrative of this invention:

#### EXAMPLES 1–20

45 Liquid admixtures were formulated from metallic mercaptans having the indicated metal content and Cab-O-Sil L-5 as an anti-agglomerant in an amount of 5% by weight of the total metal content. The liquid mixtures were then heated in open porcelain crucibles for about 3–4 hours, i.e., until a powder formed, at a temperature of 150° C. Sufficient liquid was formulated and heated for each example so that about 50 gms. of powder resulted.

50 55 60 65 The temperatures resulting were then raised in an air environment to the indicated alloying temperature and held at this temperature for the indicated period of time to insure substantially homogeneous alloying and removal of substantially all remaining organics. In some instances (where no oxidation time and temperatures are reported) oxidation was conducted simultaneously with alloying. In other instances, oxidation took place after alloying in a separate step at the indicated temperature and for the indicated period of time. In Examples 1–11 and 20 oxidation was effected before glass binder addition while in Examples 12–19, oxidation was effected after addition of the glass binder and ball milling hereinafter described.

70 75 Powder-glass binder mixtures were made by ball-milling for 96 hours at 50–50 weight percent size less than about 5 microns and consisting of by weight: 10% SiO<sub>2</sub>; 25% B<sub>2</sub>O<sub>3</sub>; 5% Al<sub>2</sub>O<sub>3</sub>; 25% ZnO; and 35% PbO. The ball-mill employed was a size 0–0 mill and milling was done with an aluminum oxide based mill and acetone. The resulting powders were then dried of acetone (and in Examples 12–19 where then oxidized) and pastes were made.

The pastes were formulated by using 3 parts by weight powder and 1 part by weight organic liquid vehicle. The organic liquid vehicle consisted of 15% by weight T-10 ethyl cellulose dissolved in 85% by weight of 2 parts by weight butyl Carbitol acetate and 1 part by weight iso-amyl salicylate.

The pastes were then printed upon 1 inch square aluminum oxide substrates using a 200 mesh stencil screen. The printed design was then air dried at about 100° C. for about 5 minutes and then fired in an open air continuous belt conveyor kiln, except in Examples 15-17 where a box kiln was used, using the indicated firing cycle. The results, reported in the following table were obtained:

said anti-agglomerating agent being selected from ultra-fine silica and an ultrafine refractory.

2. A resistor composition according to claim 1 wherein said resistive metal is palladium.

3. A resistor composition according to claim 1 wherein in said organometallic compounds are mercaptans.

4. A resistor composition according to claim 1 which includes two metal stabilizers having a metal content weight ratio selected from Ag:Au, about 4:1-1:4; Pt:Ag, about 8:1-1:8; and Pt:Au, about 8:1-1:8.

5. A resistor composition according to claim 4 wherein said resistive metal is palladium.

6. A resistor composition according to claim 1 wherein

TABLE A

| Example               | Metal wt. percent, organo metallic | Alloying temp. (° C.) | Alloying time (hrs.) | Oxidizing temp. (° C.) | Oxidizing time (hrs.) | Firing temp., ° C. (peak) | Firing time (min. at peak) | Total firing time (min.)     | Resistance K ohms/sq. p.p.m.   | TCR, p.p.m./C. |      |
|-----------------------|------------------------------------|-----------------------|----------------------|------------------------|-----------------------|---------------------------|----------------------------|------------------------------|--------------------------------|----------------|------|
| 1.....                | Pd, 65; Ag, 28; Au, 7.....         | 800                   | 16                   | 725                    | 72                    | 700                       | 5.4<br>6.0<br>6.9<br>7.0   | 21.5<br>24.0<br>27.0<br>11.0 | 10.5<br>11.0<br>11.0<br>+40    | +65            |      |
| 2.....                | Pd, 65; Ag, 28; Au, 7.....         | 725                   | 16                   | 725                    | 72                    | 700                       | 5.4<br>6.0<br>6.9<br>7.0   | 21.5<br>24.0<br>27.0<br>11.0 | 4.6<br>5.0<br>6.3<br>+25       | +200           |      |
| 3.....                | Pd, 40; Ag, 48; Au, 12.....        | 725                   | 16                   | 725                    | 72                    | 700                       | 5.4<br>6.0<br>6.9<br>7.0   | 21.5<br>24.0<br>27.0<br>11.0 | 6.0<br>6.2<br>5.8<br>+30       | +390           |      |
| 4.....                | Pd, 40; Ag, 48; Au, 12.....        | 800                   | 16                   | 725                    | 16                    | 700                       | 5.4<br>6.0<br>6.9<br>7.0   | 21.5<br>24.0<br>27.0<br>11.0 | 1.2<br>1.8<br>2.1<br>+445      | +350           |      |
| 5.....                | Pd, 60; Ag, 32; Au, 8.....         | 850                   | 8                    | 725                    | 8                     | 700                       | 5.4<br>6.0<br>6.9<br>7.0   | 21.5<br>24.0<br>27.0<br>11.0 | 2.0<br>4.0<br>5.0<br>+325      | +375           |      |
| 6.....                | Pd, 50; Ag, 40; Au, 10.....        | 725                   | 16                   | 725                    | 72                    | 700                       | 5.4<br>6.0<br>6.9<br>7.0   | 21.5<br>24.0<br>27.0<br>11.0 | 15<br>17<br>8<br>+25           | +120           |      |
| 7 <sup>1</sup> .....  | Pd, 45; Ag, 44; Au, 11.....        | 725                   | 16                   | 725                    | 72                    | 700                       | 5.4<br>6.0<br>6.9<br>7.0   | 21.5<br>24.0<br>27.0<br>11.0 | 2.5<br>2.7<br>2.7<br>+310      | +310           |      |
| 8 <sup>1</sup> .....  | Pd, 45; Ag, 44; Au, 11.....        | 700                   | 16                   | 725                    | 72                    | 700                       | 5.4<br>6.0<br>6.9<br>7.0   | 21.5<br>24.0<br>27.0<br>11.0 | 40<br>20<br>20<br>+160         | +160           |      |
| 9 <sup>2</sup> .....  | Pd, 56; Ag, 35; Au, 8.8.....       | 775                   | 16                   | 725                    | 72                    | 700                       | 5.4<br>6.0<br>6.9<br>7.0   | 21.5<br>24.0<br>27.0<br>11.0 | 2.0<br>2.0<br>2.0<br>+175      | +175           |      |
| 10 <sup>2</sup> ..... | Pd, 56; Ag, 35; Au, 8.8.....       | 775                   | 16                   | 725                    | 72                    | 700                       | 5.4<br>6.0<br>6.9<br>7.0   | 21.5<br>24.0<br>27.0<br>11.0 | 40<br>40<br>40<br>+190         | +190           |      |
| 11 <sup>2</sup> ..... | Pd, 56; Ag, 35; Au, 8.8.....       | 800                   | 16                   | 725                    | 72                    | 700                       | 5.4<br>6.0<br>6.9<br>7.0   | 21.5<br>24.0<br>27.0<br>11.0 | 1.13<br>1.13<br>1.13<br>-50    | -50            |      |
| 12.....               | Pd, 35; Ag, 52; Au, 13.....        | 800                   | 16                   | 400                    | 16                    | 710                       | 5.4<br>6<br>8<br>10        | 30<br>40<br>50<br>50         | 1.17<br>1.17<br>1.15<br>+25    | -10            |      |
| 13.....               | Pd, 35; Ag, 52; Au, 13.....        | { 800                 | 16                   | 400                    | 16                    | 710                       | 5.4<br>6<br>8<br>10        | 30<br>40<br>50<br>50         | 0.100<br>0.125<br>0.168<br>+25 | +310           |      |
| 14.....               | Pd, 35; Ag, 52; Au, 13.....        | { 725                 | 8                    | 400                    | 16                    | 710                       | 5.4<br>6<br>8<br>10        | 30<br>40<br>50<br>50         | 3.5<br>4.9<br>5<br>+315        | +315           |      |
| 15.....               | Pd, 35; Ag, 52; Au, 13.....        | 800                   | 16                   | 400                    | 16                    | 643                       | 10<br>700<br>725           | 30<br>30<br>30               | 2.5<br>1.3<br>1.8<br>+170      | 0              |      |
| 16.....               | Pd, 35; Ag, 52; Au, 13.....        | { 800                 | 16                   | 400                    | 16                    | 643                       | 10<br>700<br>725           | 30<br>30<br>30               | .390<br>.180<br>.150<br>-120   | +200           |      |
| 17.....               | Pd, 35; Ag, 52; Au, 13.....        | { 725                 | 8                    | 400                    | 16                    | 643                       | 10<br>700<br>725           | 30<br>30<br>30               | .390<br>.180<br>.150<br>-350   | +350           |      |
| 18.....               | Pd, 50; Ag, 40; Au, 10.....        | { 800                 | 16                   | 400                    | 16                    | 710                       | 5.4<br>6<br>8<br>10        | 30<br>30<br>30<br>30         | 1.5<br>.800<br>.800<br>+600    | +430           |      |
| 19.....               | Pd, 50; Ag, 40; Au, 10.....        | { 725                 | 8                    | 400                    | 40                    | 710                       | 5.4<br>6<br>8<br>10        | 30<br>30<br>30<br>30         | 1.5<br>.800<br>.800<br>+450    | +450           |      |
| 20.....               | Pd, 35; Pt, 8; Ag, 57.....         | { 800                 | 16                   | 725                    | 16                    | 700                       | 5.4<br>6<br>8<br>10        | 24                           | .0073                          | +169           | +169 |

<sup>1</sup> 48% glass binder used.

<sup>2</sup> 48.6% glass binder used.

<sup>3</sup> In run 3 insufficient alloying (too low temp. and time) was effected to achieve good reproducibility.

Once given the above disclosure, many other features, modifications and improvements will become apparent to the skilled artisan. Such other features, modifications and improvements are, therefore, considered to be a part of this invention, the scope of which is to be determined by the following claims.

We claim:

1. A resistor composition comprising a resistive metal-organometallic compound, at least one metal stabilizer in organometallic form and an anti-agglomerating agent which is inert to the system and which prevents agglomeration of the resistive metal and metal stabilizer during alloying thereof, which alloying is conducted prior to the firing of the composition into a resistor structure,

said resistive metal being selected from the group consisting of palladium, rhodium, iridium, ruthenium, indium, and mixtures thereof;

said metal stabilizer being selected from the group consisting of silver, gold, and platinum and mixtures thereof; and

the metal content of the composition is 5-95% by weight resistive metal.

7. A resistor composition according to claim 1 wherein said resistive metal is palladium and the metal content of said composition is 15-75% by weight palladium, the remainder of the metal content consisting essentially of said stabilizer metal.

#### References Cited

#### UNITED STATES PATENTS

|    |           |         |                          |         |
|----|-----------|---------|--------------------------|---------|
| 65 | 2,950,996 | 8/1960  | Place, Sr., et al. ----- | 252—514 |
|    | 3,505,134 | 4/1970  | Short -----              | 252—514 |
|    | 3,149,002 | 9/1964  | Place, Sr., et al. ----- | 252—514 |
|    | 3,248,345 | 4/1966  | Mones et al. -----       | 252—514 |
|    | 3,343,985 | 9/1967  | Vickery -----            | 252—514 |
| 70 | 3,479,216 | 11/1969 | Counts et al. -----      | 252—514 |

DOUGLAS J. DRUMMOND, Primary Examiner

U.S. Cl. X.R.